

## UNITED STATES PATENT OFFICE

2,363,984

## GASOLINE INSOLUBLE LUBRICANT

John D. Morgan, South Orange, and Russell E. Lowe, East Orange, N. J., assignors to Cities Service Oil Company, New York, N. Y., a corporation of Pennsylvania

No Drawing. Application April 17, 1943,  
Serial No. 483,462

5 Claims. (Cl. 252—41)

Our invention relates to an improved lubricant for valves or stopcocks, and more particularly to a plastic lubricant which is insoluble in gasoline motor fuels and other light hydrocarbons.

There is a considerable demand for such a lubricant particularly in the valves of apparatus used in the handling of aromatic and other gasolines, especially in aeroplane equipment which operates over a rather wide temperature range of from minus 50° F. to temperatures considerably above 100° F. Lubricants have been provided for plug cocks used in the handling of naphtha and other hydrocarbons but as far as known these lubricants are greases containing various soaps as well as solid materials such as graphite and mica.

The primary object of the present invention is to provide a lubricant which can be used in the lubrication of the moving parts of apparatus for handling light hydrocarbons and which is highly resistant to the solvent action of such hydrocarbons.

A further object of the invention is to provide an adherent valve lubricant usable in contact with light hydrocarbons and which is free of soaps and solids such as talc, graphite or mica.

Another object of the invention is to provide a lubricant which is insoluble in aromatic gasolines and which is usable in contact with such gasolines at temperatures of about minus 50° F. to 150° F.

We have discovered that a mixture of stearamide,  $\text{CH}_3(\text{CH}_2)_{16}\text{CONH}_2$ , and glycol-monophthalate-monoalphaamino stearate,



is an excellent lubricant for stopcocks and other valves or moving parts of apparatus used in the handling of gasolines and is effective over a considerable temperature range including temperatures at which aircraft operate. The features of our invention are illustrated below in connection with a specific example in which the proportions are by weight.

Commercial stearamide, 4 parts, was melted with 10 parts of commercial glycol-monophthalate-monoalphaamino stearate and thoroughly mixed and worked to produce a homogeneous solution. When this mixture or solution was cooled to room temperature it had a consistency about like that of a medium cup grease, that is an A. S. T. M. worked penetration of 155 to 200. It had a dropping point A. S. T. M. of 178° F.

and showed no corrosion in the copper strip test.

This lubricant passed the Navy test for low temperature greases which is conducted with a ball bearing tester with a torque of 3000 gm. cm. The Navy limit for a low temperature grease is 30 seconds for one revolution on this tester whereas the present lubricant at minus 40° F. showed only 4 seconds and at minus 60° F. only 5 seconds.

The solubility of the lubricant in light hydrocarbons was tested with a hydrocarbon mixture consisting of 60 per cent by volume of a commercial gasoline having an octane number of about 74, 5 percent of benzol, 20 per cent of toluol, and 15 per cent of xylol. It was found that the lubricant was insoluble in this mixture at all temperatures up to about 145° F., at which there was a very slight solubility. The solubility test with this hydrocarbon mixture is regarded as more severe than would be encountered with any commercial gasoline or other hydrocarbons, such as the butanes, propanes, Diesel fuels and naphtha.

The effectiveness of the lubricant was tested by lubricating a spring seated brass plug cock which was held in an electric oven at 165° F. until equilibrium was attained. The operation of the plug cock was found to be free and easy. The same plug cock was lubricated and tested at a temperature of minus 50° F. The cock was found to turn smoothly but was very stiff. At minus 40° F. the movement was free and smooth.

The lubricant of the present invention is not a grease but may be regarded as a solid or plastic solution which is insoluble in gasoline and other light hydrocarbons over a wide temperature range including temperatures higher than those normally encountered in the use of aircraft and other equipment in which motor fuels are handled. There may be interaction between the  $—\text{NH}_2$  of the amine and the free  $—\text{COOH}$  of the glycol ester. The consistency of the lubricant may be varied somewhat by changing the ratio of the stearamide and the glycol-monophthalate-monoalphaamino stearate to suit specific conditions or purposes. In general the ratio of the stearamide may vary from 3 to 5 parts, to 10 parts of the glycol ester, or from approximately 1:2 to 1:3.

While the specific constituents of the lubricant of the present invention provide an excellent motor fuel-insoluble lubricant it is to be understood that the use of equivalent materials comes within the scope of the present invention. Instead of using stearamide, which contains 18 carbon atoms, acid amides containing slightly more or slightly fewer carbon atoms may be employed.

Likewise the glycol ester may vary somewhat from that named above by including an amino acid group of slightly more or fewer carbon atoms than amino stearic acid. The amino group may be on a different carbon. The phthalic acid group may likewise be changed so long as the general characteristics of the mixture constituting the lubricant is not substantially altered.

The consistency of the lubricant may be changed by varying the proportions of the two constituents so as to obtain an A. S. T. M. worked penetration of from 120 to 340. Such modifications, and lubricants containing equivalent materials are intended to be covered by the appended claims.

Having described the invention in its preferred form what we claim as new is:

1. A lubricant which can be used in the lubrication of the moving parts of apparatus for handling light hydrocarbons and which is highly resistant to the solvent action of such hydrocarbons consisting essentially of a mixture of from 3 to 5 parts by weight of stearamide and 10 parts by weight of a glycol-monophthalate-monoamino stearate.

2. A lubricant which is insoluble in aromatic gasolines at the usual atmospheric temperatures and which may be used in contact with such gasolines, consisting essentially of a mixture of stearamide and glycol-monophthalate-monoalphaamino stearate in a ratio by weight of from approximately 1:2 to 1:3.

3. A valve lubricant for use in apparatus for handling gasolines and other light hydrocarbons consisting essentially of a mixture of approximately 4 parts by weight of stearamide and 10 parts by weight of glycol-monophthalate-monoalphaamino stearate.

4. A lubricant consisting essentially of from 3 to 5 parts by weight of stearamide to approximately 10 parts by weight of glycol-monophthalate-monoalphaamino stearate.

5. A lubricant consisting essentially of 4 parts by weight of stearamide and 10 parts by weight of glycol-monophthalate-monoalphaamino stearate.

JOHN D. MORGAN.  
RUSSELL E. LOWE.